

May 25, 1943.

W. MICHAELIS  
PROCESS AND ARTICLE FOR USE IN THE MANUFACTURE  
OF COMBINED PICTURE AND SOUND FILMS  
Filed July 12, 1939

2,320,005



Key:

dye.

metallic silver.

silver salt.

Inventor  
Walter Michaelis,

By Gerald Foye  
Attorney

## UNITED STATES PATENT OFFICE

2,320,005

PROCESS AND ARTICLE FOR USE IN THE  
MANUFACTURE OF COMBINED PICTURE  
AND SOUND FILMSWalter Michaelis, Brussels-Forest, Belgium, as-  
signor, by mesne assignments, to Chromogen,  
Incorporated, a corporation of NevadaApplication July 12, 1939, Serial No. 284,107  
In Germany July 13, 1938

9 Claims. (Cl. 95-2)

The present invention relates to a process for the manufacture of a combined picture and sound film in which the picture part is a multicolor image and in which the sound part consists of a metallic silver sound track on a colored or uncolored background. According to the present invention those combined picture and sound films already known as such can be manufactured in a special manner adapted to particular requirements in practice.

In the manufacture of advertising films it is customary to manufacture such advertising films whose picture part shows identically the same plot in the form of a colored cinematographic picture strip and which differ only in the accompanying text prepared especially for the businessmen of a special branch who live at different places. In the interest of economical production, it is very advantageous if such films can be manufactured in a large series and placed in reserve during times of reduction in the normal amount of work, these films having the desired text subsequently added thereto. Also in those cases in which some copies must be provided with a subsequently synchronised form in a foreign language it is desirable to manufacture the picture strips necessary for the copies in foreign language directly following the production of the large series of the actual film, even if the synchronising is not finished and hence the completion of the copies is still impossible. Finally, it lies in the interest of simplified processing to possess some finished picture strips in reserve which, in case of a sudden need can be provided with the one or the other language text. The invention fulfills these and similar requirements. It is therefore in accordance with my invention that in the picture part of the film the part images necessary for the production of the multicolor image are printed and thereafter transformed into dye images and that on the other hand, the sound strip, i. e., that part of the film into which the sound track is to be printed, is completely blackened by means of a uniform exposure and development so that after the completion of the picture part the film consists of a multicolor image and a uniformly black strip of metallic silver in the entire field of the sound track which is to be used for a later recording. For recording purposes the uniformly black strip of metallic silver is transformed into a light-sensitive salt and the light-sensitive strip thus obtained is used for printing the sound track, thereby (after exposure and fixing) yielding the black sound track. This invention described

above in its fundamental form can be carried out in many different ways these procedures varying according to the method used for the production of the dye image. Several of these procedures are described in the following.

In the accompanying drawing, Fig. 1 is a flow diagram illustrating successive sectional views of a three layer film in which the successive views represent successive stages in a processing treatment using a dye destroying process. Fig. 2 is a similar flow diagram illustrating successive stages in a processing treatment using a color development process.

*Example 1.*—Production of the multicolor image by local dye destruction. A three layer film such as shown in Fig. 1 with predyed layers 1, 2 and 3 differently sensitized according to Patent No. 2,183,393 of December 12, 1939, is used. It comprises a support 4 coated on both sides and carrying blue-sensitive layers 1 and 3 as the top and rear layers and a yellow-dyed red-sensitive layer as the middle layer 2. The part color images are printed from positive master images into the different layers, i. e., the red extract with blue light into the bluegreen layer 1, the green extract with blue light into the magenta layer 3 and the blue extract with red light into the yellow layer 2. Furthermore, the sound strip part 5 of the film is uniformly exposed to red or blue light, the choice of light depending on whether the sound track is later to be produced on a colored or a colorless background. The entire film is thereupon treated with a dye-destroying bath, such, for example, as 5% hydrogen bromide which effects the local dye destruction at the exposed places and which does not dissolve or at most only partly dissolves the silver and which forms at the places of the silver a silver salt insoluble in the treatment bath. The silver precipitate within the area of the sound track participates in this reaction and effects decoloration of the strip designated for the sound track. The film as thus exposed and developed and later treated with such a dye destroying bath is illustrated in step I of the flow diagram shown in Fig. 1. If a complete decoloration of the strip such as shown in step I is to be effected, all three layers are exposed; or of, for example, only the blue-green color is to be destroyed so that the yellow and the magenta dye remain and finally a black and red sound track is obtained, only the bluegreen side of the film is exposed. After the dye destroying treatment the metallic silver or the silver salt, if any is formed, is dissolved out in the picture part of the film, but

not in the sound track part of the film. The silver salt formed in this part is, on the contrary, re-converted into metallic silver before the film is fixed. As the process is illustrated in Fig. 1 all of the developed silver is converted to silver salt in both the picture part and the sound track part of the film (see particularly step II). The silver in the sound track part of the film is then re-converted to metallic silver as shown in step III. After the fixing as shown in step IV the film shows the finished multicolor image in the picture part and a uniform blackening of the sound area. In this state the film can be examined in the usual manner and can be stored in any way without any special precautions being necessary before the sound track is printed onto it. Before the printing of the sound track the film is led through a bath which converts the metallic silver into light-sensitive salt as shown in step V and thereafter it is exposed through the sound master image, developed and fixed to form the final print as shown in step VI.

The process described in the above example explains the method for a case in which the exposure of the film results in decoloration at the exposed places. The following serves as an example for a process in which the exposure has the effect that the exposed places appear colored in the finished film.

*Example 2.*—The sound film as shown in Fig. 2 is formed on a three-layer-film whose layers 6, 7 and 8 are coated on a support 9 and contain components for color development in the known manner. If in this case all three layers are equally blackened within the area 10 of the sound track and the sound track area is treated the same as is the picture part, dyes are then formed in all three layers during the color development. In this case the components must be chosen in such a way that the dyes formed are transparent for dark red or infrared light. If a black sound track on a red background is to be formed, then in this case only those two layers are exposed within the range of the sound track which develop in magenta and in yellow color. Moreover, the usual color development is performed with the only difference that the metallic silver developed at the same time as the dye is not removed by means of the usual Farmer's reducer, but is transformed beforehand throughout the entire film into silver chloride, as shown in step II, by treatment with a neutral copper chloride solution or (by treatment with other suitable solutions) into another silver salt which can be fixed out. The silver salt in the strip for the production of the sound track is re-converted, as shown in step III, into black silver by developers, fogging agents, or reducers before the film is fixed as shown in step IV. The film can be stored until the sound track is to be printed therein. The printing of the sound track is performed as described in Example 1 and as illustrated in steps V and VI of Fig. 2.

If a layer of a multilayer film which does not lie at the surface is exposed uniformly in the range of the sound track and if this layer is thereby reserved for the subsequent sound recording, the sound track does not lie at the surface and is protected against mechanical influences of any sort.

If further recordings, as for example, subtitles or intermediate titles which are to be only subsequently printed in are to be united with the picture part then these recordings can be printed

black onto a white or colored background in the same manner by uniformly exposing the corresponding image field parts. In this case the colored background can also be provided with a pattern if, for example, in two of the three colored layers dye images are produced during the image formation and only the third layer is uniformly blackened and reserved for the subsequent printing in of the titles.

10 After the silver deposit of the sound track is re-converted into a silver halide it can either at the same time with the re-conversion or, subsequently, be treated with the solution of a color or chemical sensitiser, for example, with a solution of 0.1 gram benzothiopseudocyanine ethyl iodide in 1 liter of water.

What is claimed is:

1. The process of producing a combined multicolor cinematographic and sound film from a multicolor picture film which has a series of multicolor pictures in the picture area suitable for projection and storage, and a silver deposit in the sound area only of said film, said deposit being of uniform density and area, which comprises converting said metallic silver within the sound area into a light-sensitive silver salt without affecting said multicolor pictures, printing the sound record into the sound area, developing the sound record and fixing the film.

20 2. A multicolor cinematographic film including a picture area and a sound area, said picture area containing therein a series of multicolor pictures suitable for projection and storage, said film containing a silver deposit in the sound area only, said silver deposit being of uniform density and area.

25 3. The process of producing a cinematographic film having a series of cinematographic picture records and a sound record in different areas thereof, which comprises printing the pictures into a silver halide emulsion within the picture area of said film, uniformly illuminating a silver halide emulsion in the sound area of said film, developing both areas of said film to form picture records in the picture area and a silver deposit uniformly covering the sound area, fixing said film to provide a finished picture record suitable for projection and storage, and subsequently reconverting the metallic silver within

30 the sound area alone into a light sensitive silver salt, printing the sound record into the sound area, developing and fixing the film.

40 4. The process of producing a cinematographic film having a series of multicolor picture records and a sound record in different areas thereof, which comprises printing the color separation records of the multicolor pictures into a silver halide emulsion within the picture area of said film, uniformly illuminating a silver halide emulsion in the sound area of said film, developing both areas of said film, converting the color separation records in the picture area of said film into multicolor images, removing the developed silver from said picture area in such a way as

45 to leave a uniform silver deposit in said sound area thereby providing a finished multicolor image suitable for projection and storage, and subsequently reconverting the metallic silver within the sound area into a light sensitive silver salt, printing the sound record into the sound area, developing and fixing the film.

50 5. The process of producing a cinematographic film having a series of multicolor picture records and a sound record in different areas thereof, which comprises printing the color separation

55 60 65 70 75

records of the multicolor pictures into a silver halide emulsion within the picture area of said film, uniformly illuminating a silver halide emulsion in the sound area of said film, developing both areas of said film, converting the color separation records in the picture area of said film into multicolor images, converting the developed silver in both the picture area and the sound area into a soluble silver salt, reconverting said silver salt in the sound area alone to metallic silver, dissolving the silver salt from the picture area of said film thereby providing a film suitable for projection and storage which has a silver deposit of uniform density in the sound area and a finished multicolor image in the picture area, and subsequently reconverting the metallic silver within the sound area into a light sensitive silver salt, printing the sound record into the sound area, developing and fixing the film.

6. The process of producing a multilayer cinematographic film having a series of multicolor picture records and a sound record in different areas thereof, which comprises printing the color separation records of the multicolor pictures in superposition into corresponding superposed and differently color-sensitized light sensitive silver halide emulsion layers on said multilayer film, uniformly illuminating the sound area of at least one of said differently color-sensitized layers, developing both areas of said film, converting the color separation records in the picture area of said film into multicolor images, removing the developed silver from said picture area in such a way as to leave a uniform silver deposit in the sound area of said one of said differently color-sensitized layers thereby providing a finished multicolor image suitable for projection and storage, and subsequently reconverting the metallic silver within the sound area into a light sensitive silver salt, printing the sound record into the sound area, developing and fixing the film.

7. The process of producing a cinematographic film having a series of multicolor picture records and a sound record in different areas thereof, which comprises printing the color separation records of the multicolor pictures into a silver halide emulsion within the picture area of said film, uniformly illuminating a silver halide emulsion in the sound area of said film, developing both areas of said film, converting the color separation records in the picture area of said film into multicolor images, removing the developed sil-

ver from said picture area in such a way as to leave a uniform silver deposit in said sound area thereby providing a finished multicolor image suitable for projection and storage, fixing, and subsequently reconverting the metallic silver within the sound area into a light sensitive silver salt, printing the sound record into the sound area, developing and fixing the film.

8. The process of producing a multilayer cinematographic film having a series of multicolor picture records and a sound record in different areas thereof, which comprises printing the color separation records of the multicolor pictures in superposition into corresponding superposed and differently color-sensitized light sensitive silver halide emulsion layers on said multilayer film, uniformly illuminating the sound area of at least one of said differently color-sensitized layers, developing both areas of said film, converting the color separation records in the picture area of said film into multicolor images, removing the developed silver from said picture area in such a way as to leave a uniform silver deposit in the sound area of said one of said differently color-sensitized layers thereby providing a finished multicolor image suitable for projection and storage, fixing, and subsequently reconverting the metallic silver within the sound area into a light sensitive silver salt, printing the sound record into the sound area, developing and fixing the film.

9. The process of producing a cinematographic film having a series of multicolor picture records and a sound record in different areas thereof, which comprises printing the color separation records of the multicolor pictures into a silver halide emulsion within the picture area of said film, uniformly illuminating a silver halide emulsion in the sound area of said film, developing both areas of said film, converting the color separation records in the picture area of said film into multicolor images, removing the developed silver from said picture area in such a way as to leave a uniform silver deposit in said sound area in the uniformly illuminated emulsion thereby providing a finished multicolor image suitable for projection and storage, and subsequently reconverting the metallic silver within the sound area into a light sensitive silver salt, printing the sound record into the sound area, developing and fixing the film.

WALTER MICHAELIS.